

## UNITED STATES PATENT OFFICE

2,037,937

SAFETY PAPER AND METHOD OF  
MAKING SAME

Francis L. Simons, Needham, Mass., assignor to  
George La Monte & Son, Nutley, N. J., a cor-  
poration of New Jersey

No Drawing. Application May 9, 1933,  
Serial No. 670,210

28 Claims. (Cl. 91—67.95)

This invention relates to safety paper, including fraud preventing writing material made of paper or other substance or composition adapted for printing or lithographing or for the inscription of writing thereon and for use, for example, in the manufacture of checks, drafts, bonds, stock certificates, or other instruments, which it is desired to have protected against fraudulent alteration. This invention also relates to methods of making such paper.

This invention relates particularly to safety paper manufactured using a ferrocyanide as a safety chemical.

Ferrocyanides when incorporated in safety paper have the property of forming with iron compounds in ink certain deeply colored compounds known as "Prussian blue", the exact chemical nature of which is not certain and may vary to some extent depending upon the proportions and character of the reacting substances. Prussian blue is highly resistant to the ink eradicator in general use at the present time. The most commonly used ink eradicator has a chlorine bleach as a basis. Another type of eradicator has potassium permanganate as a basis. The latter eradicator is normally followed in actual use by the application of some reducing agent such as sodium bisulphite to clean up the manganese dioxide deposited during the application of the permanganate. The Prussian blue formed by writing with ordinary iron-containing ink on safety paper prepared with ferrocyanides is resistant to the action of both of the eradicators referred to. Moreover, upon the application of acids to safety paper thus prepared, as, for example, in treating ink preliminarily for the subsequent application of a chlorine bleach type of eradicator, the ferrocyanide is caused to decompose with the formation of Prussian blue as an indelible disfiguring mark or stain. Such fraud preventing characteristics of ferrocyanides are afforded when ferrocyanides are applied to safety paper in effective amount as an ink fixing agent.

Safety papers containing soluble ferrocyanides, are subject, however, to the very serious defect that they gradually become discolored in the presence of air and/or light to produce prematurely objectionable stains and discolorations on safety paper. The discoloration of the ferrocyanide is believed to be due to a gradual decomposition of the ferrocyanide with resulting liberation of iron compounds that in turn react with the remainder of the ferrocyanide forming Prussian blues or other colored compounds. While the decomposition of the ferrocyanide and re-

sultant discoloration can be inhibited to a certain extent by the inclusion of alkali or alkaline substances in safety paper, the presence of the alkali in the paper results in almost complete loss of the sizing and waterproof characteristics of the paper. The rosin which is normally used in sizing paper is acid in character and even in the presence of weak alkali its sizing ability is promptly destroyed with the result that the sheet becomes absorbent, causing blotting and "feathering" of ink applied thereto. Moreover, alkali is not a wholly satisfactory stabilizer, as a sheet of paper treated with a soluble ferrocyanide and an alkali will eventually turn blue on standing, or in light, or more rapidly when subjected to both conditions. While attempts have been made to overcome the desizing effect of alkaline stabilizers by the use of secondary sizing materials such as starch, casein, and glue, such attempts have not resulted in commercially satisfactory products. It is a feature of this invention that it is not necessary to use a secondary sizing material to counteract any desizing effect such as would be caused by alkaline stabilizers.

It is a purpose of this invention to afford a ferrocyanide safety-paper which is satisfactory from the point of view of its resistance to discoloration upon aging in air and/or upon exposure to strong light and which is also satisfactory from the point of view of its writing properties.

According to this invention, a ferrocyanide safety paper is afforded which does not blot or cause "feathering" when ink is applied thereto and which is more perfectly protected against discoloration than any which has been manufactured heretofore.

The ferrocyanides which are particularly susceptible to decomposition are the water soluble ferrocyanides, namely, the ferrocyanides of alkali metals (including ammonium) and of alkaline earths. Such ferrocyanides will be referred to herein as soluble ferrocyanides. The use of soluble ferrocyanides is preferable in the practice of this invention because they are capable of ready application to safety paper and because they are much more effective in fixing ink applied to safety paper than are the insoluble ferrocyanides. The ferrocyanides of sodium or potassium are regarded as being particularly effective and are relatively inexpensive.

To afford a clear understanding of this invention, it will now be described in connection with certain specific examples illustrative thereof.

In one embodiment of this invention, safety

paper is manufactured which has incorporated therein not only a soluble ferrocyanide but also a substantial amount of alkali metal phosphate. The phosphates of alkali metals (including ammonium phosphate) have been found to possess the property of exerting a specific retarding effect in a very marked degree upon the decomposition of the ferrocyanide as applied to safety paper. From the point of view of both effectiveness and economy, the employment of the phosphates of sodium and potassium is regarded as preferable according to this invention.

It is one of the features of this invention that a stabilizer for preventing the decomposition of soluble ferrocyanide in safety paper is afforded which is relatively neutral. In this regard, it is to be noted that the alkali metal phosphates occur in three different forms. This may be illustrated in connection with the sodium phosphates, for example. Tri-sodium phosphate in aqueous solution shows a definitely alkaline reaction. It has been pointed out above that definite alkalinity tends to destroy the sizing of paper to a certain extent and causes ferrocyanide in safety paper to become yellow on exposure to strong light. In the case of the tri-sodium phosphate, however, increased stabilization is afforded as the phosphate radical has a specific retarding effect on the decomposition of soluble ferrocyanide. This is evidenced by the fact that tri-sodium phosphate exerts a decidedly greater retarding effect on the decomposition of soluble ferrocyanide than do other substances of equal alkalinity.

The mono-sodium phosphate has a slightly acid reaction in aqueous solution. The acidity of the mono-sodium phosphate causes ferrocyanide in safety paper to turn blue or green on ageing to a slight extent. But in this case also the phosphate radical has been found to exert a definite retarding effect in the decomposition of ferrocyanide in safety paper.

Di-sodium phosphate when made into an aqueous solution containing about 5% to about 20% of the salt has been found to have a pH value of about 8. Thus the solution is only very slightly alkaline. However, all alkalinity (and tendency to destroy the sizing of paper) can be removed by the addition to the solution of di-sodium phosphate, an acidic substance, e. g. mono-sodium phosphate or phosphoric acid. Thus, the pH value of the solution can be reduced to about 7.2, which indicates a practically neutral solution.

With a neutral solution of alkali metal phosphate, it has been found that soluble ferrocyanide in safety paper is rendered very stable both in its resistance to aging, and in its resistance to the action of strong light. While it is preferable to employ alkali metal phosphates in safety paper in as nearly a neutral condition as possible, the employment of alkali metal phosphates generally, has been found to give improved stability to ferrocyanide under both slightly acid or slightly alkaline conditions, and is to be regarded as coming within the scope of this invention. The alkali metal phosphates are specific inhibitors of photochemical decompositions of ferrocyanides and decompositions resulting from aging. Moreover, the adjusting of any of the alkali metal phosphates or mixtures thereof to a more neutral condition in safety paper is to be regarded as within the scope of this invention.

Safety paper prior to treatment with ferrocyanide solution and with alkali metal phosphate, is normally slightly acid due largely to the acidity of the sizing material. Thus, for example, the

paper by itself may have a pH value of about 4.7 to about 6.5. In such case when the paper is treated with a solution of alkali metal phosphate adjusted to a pH value of about 7.2 to about 7.5 the resulting paper after drying will be found to be very slightly acid and may have a pH value of about 6.5 to about 7.0 and such conditions in the finished safety paper are regarded as preferable. In the practice of this invention the pH value of the finished paper may range between about 6.2 and about 7.3 with very satisfactory results.

As a specific illustration of this invention, a bath is made up containing 10% sodium ferrocyanide, 12% di-sodium phosphate and 1% mono-sodium phosphate, the balance of the solution being water. The proportions given are based upon the weight of the fully hydrated commercial salts that are added to the impregnating bath. The acidity of the solution thus made up is in the neighborhood of 7.5 on the pH scale. The solution can be applied in the manufacture of safety paper in any suitable manner. For example, the paper can be passed through a bath of the solution and then subjected to squeeze rolls to squeeze out excess moisture. The paper thus treated can then be dried and finished in any suitable manner, as is well known in the art.

Due to the fact that the paper itself is slightly acid as stated above, the finished paper will be very nearly neutral. As the bath becomes depleted, it, of course, can be renewed as the needs require. In this connection, it has been found that the bath takes up a slight degree of acidity from the paper and to offset this it is preferable to replenish the bath with a solution which has a pH value that is about .2 to about .3 higher than pH value desired in the bath that is applied directly to the paper.

While it is normally preferable to apply the solution uniformly throughout the body of the sheet in the manner above described, the solution can, of course, be applied in any other manner as by spraying the sheet with the solution, applying the solution locally as by printing or otherwise, or in any other suitable manner. Moreover, the ferrocyanide and stabilizer therefore can both be applied together in a single impregnating bath or can be applied separately as by separate baths. Whether the ferrocyanide and/or stabilizer therefor are applied through the material or at the surface, the same will be regarded as incorporated with the safety paper.

It is to be noted that the above solution contains a substantial quantity of di-sodium phosphate and substantial quantity of mono-sodium phosphate. The mixture of the two phosphates or of the phosphates with phosphoric acid in the finished paper has been found to act in the capacity of an acid-alkali buffer giving increased resistance to the action of acids or alkalies. Thus, the finished paper is not easily discolored by air containing gases such as  $\text{SO}_2$  or by waste gases of acid or alkaline nature. The inclusion of such buffer with the safety paper is to be regarded as an advantage and feature of this invention. Moreover, the presence of the buffer in the impregnating bath contributes to the maintenance of uniform alkali-acid conditions which otherwise might be affected to undesirable extent by such causes as bringing different rolls of paper having different degrees of acidity into the bath. Another buffer combination is a solution of mixed sodium sulphite and sodium bi-sulphite. The

latter substances also exhibit some stabilizing effect on ferrocyanides, as well.

To give another specific example of an application of this invention, an impregnating bath is made up containing 7.5% of potassium ferrocyanide, 15% di-sodium phosphate and about 1% of phosphoric acid, the balance being water. In the illustration just given, the phosphoric acid is used to reduce the normal alkalinity of di-sodium phosphate solution to approximately the neutral point. This impregnating bath may be applied in the manufacture of safety paper as above described.

Alkali metal ferrocyanides are practically neutral in themselves. Thus the chemical substances incorporated in the safety paper including both the ferrocyanide and the protecting agent therefore, in the above specifically illustrating embodiments of this invention, are, taken altogether, about neutral.

Preferred results can be produced in the practice of this invention by controlling the pH value of the incorporated substance between 6.8 on the acid side and about 7.5 on the alkaline side. However, the advantages of this invention resulting from keeping the impregnated material at about the neutral point can be largely afforded by controlling the pH value of the incorporated substances between about 6.7 on the acid side and about 8.5 on the alkaline side.

In preparing safety paper with ferrocyanide, it is usually preferable to employ enough of the ferrocyanide to exhibit a pronounced ink fixing reaction with the iron in inks which may be applied thereto and to give a pronounced discoloration if acids are applied to the paper. The employment of a solution of ferrocyanide of approximately 10% concentration will afford a bath which will incorporate in the safety paper a suitable amount of ferrocyanide to produce the desired protection. The finished paper usually contains about  $\frac{1}{5}$ th the proportion of ferrocyanide and stabilizing agent which is contained in the impregnating bath. Usually about  $\frac{1}{2}\%$  to about 2% of ferrocyanide should be incorporated in the manufactured safety paper to impart very pronounced fraud preventing characteristics to the paper. The amount of ferrocyanide that is incorporated in the paper may be increased to about 5% which approaches the maximum amount that the paper will retain when impregnated with a saturated solution of ferrocyanide. The more ferrocyanide that is retained in the paper the more vigorous the ink fixing and stain producing reactions become. It is a feature of this invention that the ferrocyanide is stabilized to a commercially satisfactory extent even though a maximum amount of ferrocyanide is incorporated in the safety paper. For purposes of economy, lesser quantities of ferrocyanide such as the quantities above suggested may be used and have been found to give satisfactory ink fixing and stain producing properties to safety paper.

The amount of alkali metal phosphates which should be used to stabilize the ferrocyanide is subject to considerable variation. More than about 5% by weight in the bath of the alkali metal phosphate should preferably be added to a 10% solution of ferrocyanide to give desired stability to the ferrocyanide in the finished paper as the amount of phosphate stabilizer should preferably be not less than about half the amount of ferrocyanide to afford satisfactorily permanent stabilization. Preferably the amount of alkali metal phosphate used should be about 50% to

150% on the weight of the ferrocyanide. Increased amounts of the phosphates give greater stability. There is probably no precise upper limit as to the amount of phosphate which may be used except that by the use of excessive amounts of phosphate, the cost of the safety paper may become unnecessarily increased. Usually about 12% to about 14% of alkali metal phosphate in a 10% solution of sodium ferrocyanide gives very excellent stabilization of the ferrocyanide and safety papers made from such an impregnating bath not only exhibit in high degree the safety features of ink fixing and stain production but also are highly resistant to subsequent discoloration due to decomposition of the ferrocyanide.

A safety paper containing ferrocyanide, stabilized by alkali metal phosphates can be further improved by incorporating in the safety paper an alkali metal fluoride, e. g. sodium fluoride. Alkali metal fluoride exhibits the property of preventing iron compounds which result from the decomposition of ferrocyanide in safety paper, from reacting with undecomposed ferrocyanide and forming colored compounds. Thus the alkali metal fluorides have to a considerable degree the capacity of stabilizing ferrocyanides. While the employment of alkali metal fluoride with sodium phosphate is desirable in the practice of this invention, the employment of alkali metal fluoride alone as a stabilizer for ferrocyanide in safety paper is to be regarded as one of the features of this invention.

When sodium fluoride, for example, (which in itself is approximately neutral) is used in connection with the employment of alkali metal phosphates to stabilize ferrocyanide in safety paper, the employment of a bath having slightly greater acidity than would be possible in the absence of sodium fluoride, is permissible. Thus a fairly high degree of protection against discoloration caused by decomposition of ferrocyanide can be afforded by adding about 1% of sodium fluoride to the impregnating baths given in the foregoing illustrations of the practice of this invention even though the pH value of the bath is as low as about 6. In the finished paper the pH value, when an alkali metal fluoride is used, preferably ranges from about 6 to 7.1.

The amount of alkali metal fluoride which need be used in the practice of this invention is relatively small. For example, about 1% of sodium fluoride in a bath which is applied to the paper is sufficient to give the desired results. Lesser quantities give decreasing stabilizing effect. Greater quantities do not result in substantially greater stabilizing effect. Moreover, it is ordinarily preferable to employ less than about 0.5% of alkali metal fluoride as the employment of substantially greater quantities than 1% in the bath results in a slight and gradual desizing effect in the finished paper.

While it is regarded as preferable to employ alkali metal phosphates as stabilizing agents in preventing the decomposition of ferrocyanide in safety paper, it has been found according to this invention that considerable stabilizing effect is afforded by employing in a substantially neutral solution the salts of alkali metals and alkaline earths, both inorganic such as chlorides, sulfates, borates, etc. and organic such as citrates, benzoates, salicylates and the like. For use in connection with safety paper, it is of course desirable that the salt used be substantially colorless unless a paper corresponding to the color of the

salt be used or unless the color is suitably camouflaged or is regarded as desirable. It is to be understood that ammonium salts are not included among the alkali metal and alkaline earth salts other than phosphates which may be employed according to this invention.

If any of the salts above mentioned which may be used according to this invention either have a definitely acid or definitely alkaline reaction, their alkaline or acid characteristics should be neutralized so as to bring the pH value of the solution thereof within about 6.7 on the acid side and about 8 on the alkaline side, except that when the alkali metal fluoride is used with any of the salts, the resulting solution can be used in a somewhat more acid state, namely, having the pH value above about 6. Moreover, such salts should not react with the ferrocyanides as by causing the oxidation or reduction of the ferrocyanides.

When other alkali metal or alkaline earth salts are used than alkali metal phosphates (which latter are regarded as preferable) relatively large quantities of the salts should be used to produce substantial stabilization of the ferrocyanide. About 50% to 150% of such salts in proportion to the weight of the ferrocyanide should preferably be incorporated in the paper. The pH value of the finished paper should preferably be about 6.2 to about 7.3.

This invention has heretofore been described in connection with the stabilization of soluble ferrocyanides employed in connection with safety paper. If an insoluble ferrocyanide is employed, such as manganese ferrocyanide as by the precipitation of manganese ferrocyanide from a solution of soluble ferrocyanide incorporated with the paper, such paper can be greatly improved by employing the stabilizing chemicals hereinabove described. In the method of preparing safety paper using an insoluble ferrocyanide formed by impregnation with successive baths, it is difficult to bring about complete interaction between the soluble ferrocyanide and the soluble manganese salt, whereby free soluble ferrocyanide is frequently left in the paper. The incorporation of the stabilizing chemical hereinabove described serves to prevent the discoloration of the safety paper due to the decomposition of otherwise spontaneously decomposable ferrocyanide in the safety paper.

While this invention has been described in connection with certain specific examples thereof, it is to be understood that this has been done for the purpose of illustration and that the scope of this invention is not to be limited thereby. It is also to be understood that this invention is capable of other applications than those herein given by way of illustration.

60 I claim:

1. As an article of manufacture, a safety paper having incorporated therewith a ferrocyanide and an alkali metal phosphate.
2. As an article of manufacture, a safety paper having incorporated therewith a soluble ferrocyanide and an alkali metal phosphate.
3. As an article of manufacture, a safety paper having incorporated therewith a soluble ferrocyanide and a substance selected from the group consisting of sodium and potassium phosphate.
4. As an article of manufacture, a safety paper having incorporated therewith a ferrocyanide, an alkali metal fluoride, and an alkali metal phosphate.
5. As an article of manufacture, a safety paper

having incorporated therewith a soluble ferrocyanide, sodium fluoride, and a substance selected from the group consisting of sodium and potassium phosphate.

6. As an article of manufacture, a safety paper having incorporated therewith a ferrocyanide and an alkali metal fluoride.

7. As an article of manufacture, a safety paper having incorporated therewith a soluble ferrocyanide and a substance selected from the group consisting of sodium and potassium fluoride.

8. As an article of manufacture, a safety paper comprising a soluble ferrocyanide and an alkali metal phosphate, the pH value of the finished product being between about 6.2 and about 7.3.

9. As an article of manufacture, a safety paper comprising a soluble ferrocyanide and a substance selected from the group consisting of sodium and potassium phosphate, the pH value of the finished product being between about 6.5 and about 7.0.

10. As an article of manufacture, a safety paper comprising a soluble ferrocyanide, sodium fluoride, and a substance selected from the group consisting of sodium and potassium phosphate, the pH value of the substances embodied in said sheet being between about 6.0 and about 7.1.

11. As an article of manufacture, a safety paper containing a soluble ferrocyanide, and di-sodium phosphate.

12. As an article of manufacture a safety paper comprising a soluble ferrocyanide, di-sodium phosphate, and mono-sodium phosphate.

13. As an article of manufacture, a safety paper comprising a soluble ferrocyanide and an acid-alkali buffer, the pH value of the finished product being between about 6.2 and about 7.3.

14. As an article of manufacture, a safety paper comprising a soluble ferrocyanide and a substance selected from the group consisting of soluble salts of alkaline earth metals and of alkali metals other than an ammonium, the pH value of the finished product being between about 6.2 and about 7.3.

15. As an article of manufacture, a safety paper comprising a ferrocyanide, sodium fluoride and a colorless soluble salt of an alkali metal, the pH value of the substances incorporated in said sheet being between 6.0 and 7.1.

16. As an article of manufacture, a safety paper comprising incorporating therewith about 1/2% to about 5% of a soluble ferrocyanide and an alkali metal phosphate, the amount of alkali metal phosphate being about 50% to about 150% of the weight of the ferrocyanide.

17. As an article of manufacture, a safety paper comprising a soluble ferrocyanide and a substance selected from the group consisting of sodium sulphite and sodium bisulphite the pH value of the finished product being between about 6.2 and about 7.3.

18. A method of making safety paper which comprises incorporating with the paper water-dissolved ferrocyanide and a water-dissolved salt of a metal selected from the group consisting of alkaline earth metals and alkali metals other than ammonium, the pH value of the dissolved substances applied to the paper being between about 6.7 and about 8.5 and removing excess water.

19. A method of making safety paper which comprises incorporating with the paper water-dissolved ferrocyanide and a water-dissolved salt of a metal selected from the group consisting of alkaline earth metals and alkali metals other than ammonium, the pH value of the dissolved substances applied to the paper being between about 6.7 and about 8.5 and removing excess water.

than ammonium, the pH value of the dissolved substances applied to the paper being between about 6.7 and about 8.5 and removing excess water, the pH value of the paper prior to the application of said dissolved substances thereto being between about 4.7 and about 6.5.

20. A method of making safety paper which comprises incorporating with paper water-dissolved ferrocyanide and water-dissolved alkali metal phosphate and removing excess water.

21. A method of making safety paper which comprises incorporating with paper water-dissolved ferrocyanide and water-dissolved alkali metal phosphate, the pH value of the dissolved substances as applied to the paper being between about 6.8 and about 8.

22. A method of making safety paper which comprises incorporating with paper water-dissolved ferrocyanide and water-dissolved alkali metal phosphate, the pH value of the dissolved substances as applied to the paper being between about 6.8 and about 8, the pH value of the paper prior to the application of said dissolved substances thereto being between about 4.7 and about 6.5.

23. A method of making safety paper which comprises incorporating with paper water-dissolved ferrocyanide and water-dissolved di-alkali metal phosphate and removing excess water.

30. 24. A method of making safety paper which comprises incorporating with paper water-dissolved ferrocyanide and a water-dissolved mixture of di-sodium phosphate and phosphoric acid and removing excess water.

25. A method of making safety paper which comprises incorporating with paper water-dissolved ferrocyanide and a water-dissolved mixture of di-sodium phosphate and mono-sodium phosphate and removing excess water.

5

26. As an article of manufacture, a safety paper comprising a soluble ferrocyanide, a size decomposable in the presence of a substantial amount of alkali, and a stabilizer for ferrocyanide, the pH value of the finished product being between about 6.2 and about 7.3.

27. As an article of manufacture, a safety paper comprising a soluble ferrocyanide and an acid alkali buffer including sodium sulphite and sodium bisulphite the pH value of the finished product being between about 6.2 and about 7.3.

28. A method of making safety paper which comprises incorporating with the paper water-dissolved ferrocyanide and as a stabilizer for the ferrocyanide a water-dissolved salt of a metal selected from the group consisting of alkaline earth metals and alkali metals other than ammonium, the pH value of the bath of dissolved substances applied to the paper being between about 6.7 and about 8.5 and removing excess water, the pH value of the paper prior to the application of said dissolved substances thereto being between about 4.7 and about 6.5, and replenishing the impregnating bath with fresh quantities of dissolved ferrocyanide and dissolved stabilizer, the pH value of replenishing materials being about .2 to about .3 greater than the bath.

FRANCIS L. SIMONS.